

## UNITED STATES PATENT OFFICE

LYNN A. WATT, OF WEBSTER GROVES, MISSOURI, ASSIGNOR TO MONSANTO CHEMICAL WORKS, OF ST. LOUIS, MISSOURI, A CORPORATION OF MISSOURI

## LEATHER DYE

No Drawing.

Application filed May 7, 1927. Serial No. 189,745.

This invention relates to leather dyes of the kind that are used for dyeing shoes.

The conventional shoe dye contains aniline or nitrobenzene, which is used principally as a penetrant or vehicle to carry the dye solution through the finish of the leather into the pores of the leather. These substances are highly toxic, and many cases of aniline or nitrobenzene poisoning, resulting in severe illness and death, have been traced directly to the practice of dyeing shoes while on the feet of a person and the practice of wearing shoes within a few hours after they have been dyed with a dye containing aniline or nitrobenzene.

The main object of my invention is to provide a non-toxic leather dye that can be used with perfect safety for dyeing shoes while they are on a person's feet.

Another object is to provide an efficient, non-poisonous shoe dye that can be manufactured at a low cost.

To this end I have devised a leather dye, particularly adapted for use in dyeing shoes, which is distinguished from conventional shoe dyes, in that a non-toxic substance is used as the penetrant or vehicle to carry the dye solution into the pores of the leather.

I have found that the dichlorbenzenes are well adapted for this purpose, the substance that I prefer to use as the penetrant for the dye solution consisting of orthodichlorbenzene or orthodichlorbenzene containing some paradichlorbenzene. When a mixture of said substances is used it is preferable to have the orthodichlorbenzene predominate in the mixture.

In addition to being non-toxic, substances of the kind mentioned are easy to obtain and are relatively inexpensive, as either orthodichlorbenzene or orthodichlorbenzene containing some paradichlorbenzene, are produced in the manufacture of monochlorbenzene, an intermediate chemical, or paradichlorbenzene, an important insecticide. No adequate market for the ortho isomer alone or containing some residual paradichlorbenzene has existed, and it is therefore available as a by-product at prices comparable with or lower than the aniline or nitrobenzene heretofore

used as the penetrant or vehicle of shoe dyes.

In producing my improved leather dye any suitable solvent for the dye may be used, such as denatured ethyl alcohol. Any suitable type or kind of dye may be used, and any suitable oil or other fatty or waxy ingredient may be used. Moreover, the proportions, percentages and strength of the various ingredients comprising the finished product may be varied over a considerable range without departing from the spirit of my invention. The following is one formula that may be used to produce my improved, non-toxic leather dye:

Orthodichlorbenzene, approximately 30.0 grams;

Spirit soluble nigrosine, approximately 7.5 grams;

Red oil (oleic acid), approximately 5.0 grams;

Denatured ethyl alcohol, sufficient to make, approximately 100.0 cc.

Having thus described my invention, what I claim as new and desire to secure by Letters Patent is:

1. A leather dye composition containing a dichlorbenzene capable of carrying a dye solution into the pores of the leather.

2. A leather dye composition including, as one of its constituents, orthodichlorbenzene.

3. A composition for the treatment of leather containing a leather dye material and at least one dichlorbenzene.

4. A leather dye composed of the following ingredients mixed in approximately the proportions specified:

Orthodichlorbenzene ----- 30.0 grams

Spirit soluble nigrosine ----- 7.5 grams

Red oil (oleic acid) ----- 5.0 grams

Denatured ethyl alcohol sufficient to make ----- 100.0 cc.

LYNN A. WATT.